

## UNITED STATES PATENT OFFICE

2,028,846

## CELLULOSE PULP FOR ESTERIFICATION PURPOSES AND PROCESSING OF SAME

George A. Richter, Berlin, N. H., assignor to Brown Company, Berlin, N. H., a corporation of Maine

No Drawing. Application June 22, 1931,  
Serial No. 546,151

2 Claims. (Cl. 260—100)

The subject of this invention is a pulp for viscose syrups and the like, as well as the processing which the pulp undergoes in passing from its original condition to the ultimate syrup or generic product. In making viscose syrups, such as are spun into artificial silk, it is the practice to use soft-wood pulps as the cellulosic base, for such pulps are convertible into syrups having the desired characteristics. It is practically impossible to realize satisfactory viscose syrups from hardwood pulps, doubtless on account of the excessive pentosans, resins, and other objectionable non-alpha-cellulose components present in such pulps even when they have been prepared by the sulphite process of fiber liberation, which, as is well known, is conducive to pulps of comparatively low pentosan content. Indeed, a sulphite pulp derived from hard woods of the character of birch, beech, and maple may have a pentosan content ranging from 5% to 7%, or even higher; yet, for economical reasons, for instance the lower cost of hard woods, the much higher yield of pulp per cord of wood, etc., the pulpmaker would like to market a product derived from hard wood, such as birch, rather than one procured from soft wood, such as spruce.

I have found that hardwood pulps, notably hard-wood sulphite pulp, may be made to fulfill the requirements for xanthation and the like, if such pulps are subjected to the action of a mercerizing liquor, preferably in the presence of an oxidant, for a sufficient period of time to remove pentosans, resins, and other non-alpha celluloses, in such amount as to leave a fiber residuum having an alpha cellulose content of at least about 94% and a pentosan content of not greater than about 1.5%. Aside from the purifying action exercised by the liquor on the pulp serving as the starting material, the liquor functions simultaneously to reduce the solution viscosity of the fiber so drastically that the mercerized fiber residuum, after washing, can be xanthated directly and completely without requiring the usual intermediate long-time ageing of the soda cellulose into which it is transformed as part of the xanthating process. The mercerizing liquor thus performs two offices on the pulp at the same time; and the pulp may be admixed with the mercerizing liquor in the same bulk condition as it was liberated in the pulp mill, as the handling of the flowable pulp suspension thus produced is easy, inexpensive, and conducive to a uniform product. The mercerizing liquor may be of varying causticity, depending upon the temperature at which it is used, for, as is well known, mercerization can be re-

alized at lower temperatures with weaker solutions of caustic soda than those necessary at higher temperatures. In fact, the liquor may be used at or below freezing temperatures, as disclosed in my application Serial No. 538,132, filed May 18, 1931 (now Patent No. 1,859,891, dated May 24, 1932), in which case, the liquor may, for instance, be caustic soda solution of only 5% strength applied at, say, 0° C., together with the desired amount of hypochlorite or other oxidant. So, too, the oxidant content of the solution may be varied, depending upon such factors as the particular oxidant used, the solution viscosity of the pulp serving as the starting material, the temperature of treatment, etc. Because the oxidant is used with a large excess of alkali, its tendency to degrade the pulp by causing the formation of oxycelluloses is almost entirely inhibited. In contrast with the mercerizing action, the activity of the oxidant is greater at higher temperatures than at lower temperatures, wherefore, to secure a given effect through the use of oxidant at, say, room temperature (20° C.), it is necessary to use more oxidant than at below room temperature, say, 10° C.

As a specific example of procedure falling within the purview of the present invention, I may cite the following. I take a birch sulphite pulp, either in bleached or unbleached condition and containing, say, 5% to 7% pentosans, and mix it with a caustic soda solution of upwards of 15% strength at room temperature to produce a stock density of, say 5% to 10%. In some cases, the hardwood pulp may be advantageously pretreated with chlorine water, hypochlorite bleach liquor, or the like, and then washed to remove some of the lignous and other coloring matter which it would otherwise be necessary to eliminate as by the addition of bleach to the mercerizing liquor with which the pulp is subsequently treated. Some types of hardwood pulp may to advantage undergo an initial treatment with a weak acid solution or other reagent to facilitate the procurement of a finished product of especially low solution viscosity. The solution should preferably contain an oxidant in amount sufficient to reduce the solution viscosity of the pulp to the desired value while it is being refined,—say, 1% to 10% hypochlorite bleach (either sodium or calcium base), or 1% to 3% potassium permanganate. The oxidant also tends to remove residual lignous and coloring matter from the pulp, and thus to whiten it. Considerably less permanganate than hypochlorite bleach need be used for bringing about a given solution-viscosity-lowering effect,

5

10

15

20

25

30

35

40

45

50

55

because of the greater activity of the permanganate on the fiber, especially under strongly alkaline conditions. After remaining suspended in the mercerizing liquor containing the oxidant for about 2 to 8 hours or more, the pulp is washed free from liquor. The washed pulp, when tested, exhibits an alpha cellulose content of at least about 94% and a pentosan content not exceeding 1.5%. When insufficiently white, it may be post-bleached to the desired whiteness under conditions to preserve its high alpha cellulose content. For instance, in case a raw or unbleached pulp has undergone processing as described but has not acquired the desired whiteness during mercerization, it may be treated, after washing, with a hypochlorite bleach liquor of sufficient potency to ensure the desired whiteness of product. The bleach liquor should also contain sufficient free alkali, such as caustic soda, sodium carbonate, or the like, to maintain a condition of appreciable alkalinity therein throughout the bleaching operation, as the free alkali preserves the previously-attained alpha cellulose content in the pulp. The washed, and, if desired, post-bleached pulp is then converted into viscose syrup substantially in the following manner. The pulp in sheet or other suitable form is treated with excess caustic soda solution of about 18% strength, and is then squeezed to the caustic soda content necessary for combining with the fiber as so-called soda cellulose. The soda cellulose is then shredded, as usual, but rather than undergoing the conventional ageing under controlled temperature conditions for a considerable period of time, the shreds may be at once treated with carbon bisulphide in amount calculated to form viscose syrup. As already stated, the soda cellulose dissolves completely to form syrup of excellent clarity, color, and viscosity for spinning into silk and for fabrication into pellicles or other viscose ultimates.

The hardwood pulp product of the present invention, while especially adapted for making xanthates or other esters, is by itself poorly adapted for papermaking. To begin with, it must be borne in mind that a hardwood pulp, since as birch sulphite pulp, is characterized by a much shorter average fiber length than is spruce sulphite pulp. Mercerization further impairs the fiber for papermaking, because it destroys the ability of the fiber to become hydrated during beating, and thus to furnish strengthening gel for the paper. Then, too, a mercerized fiber tends to clump or aggregate, with the result that it is difficult to secure uniform felting or texture on the paper machine. The fact that my product is of short average fiber length and is mercerized does not, however, militate against its utility for xanthation or other esterifying treatment, but rather inures to its benefit, for its short fiber length means smaller units, which lend themselves to more uniform treatment with converting chemical and to a quicker conversion, and its mercerized state goes hand in hand with a better composition and lower solution viscosity. The viscose syrups that are prepared from the specially treated hardwood pulp product of the present invention have exceptional clarity and are very easily filtered,—properties of great importance in the manufacture of rayon.

My invention comprehends the processing of various kinds of pre-liberated hardwood pulps, but it is more particularly aimed at such pulps which have been pre-liberated by the sulphite process of cooking. The combination of the sulphite process of cooking the raw wood to produce

pulp with the mercerizing step of the present invention makes possible an almost complete removal of the pentosans, which may be present to the extent of 20%, or even higher, in the raw wood, and which are highly detrimental to the preparation of viscose syrups or other esters of usefulness. In liberating pulp from the raw hardwood by the sulphite process, one may use the typical acid sulphite cooking liquors containing sodium or calcium as the base and having 1% or more combined  $\text{SO}_2$  and 5% or more free  $\text{SO}_2$ . The use of an acid sulphite cooking liquor containing a large excess of free over combined  $\text{SO}_2$  is of value, in that the acid sulphite cook itself removes most of the pentosans, and thus leaves less work to be done by the mercerizing treatment of the present invention. The process of the present invention can be applied to alkaline-cooked hardwood pulps—for instance, such pulps as are obtained by cooking hardwood chips in kraft or soda liquors. The pulps that are produced by such processes are higher in their pentosan content than sulphite pulp produced from the same wood. They are, therefore, even more difficult to convert into a product suitable for viscose-making or the like, unless the process of the present invention is invoked. Thus, a kraft hardwood pulp may have a pentosan content ranging from 15% to 20%. Such a raw pulp, after a suitable pre-treatment with, say, 2% to 4% chlorine, based on pulp, in the form of chlorine water, followed by washing and treatment with a mercerizing liquor containing a suitable amount of hypochlorite bleach or its equivalent as hereinbefore described, yields a product that responds to xanthation or other esterifying reaction very nicely.

The main treatment of the pulp with mercerizing liquor may advantageously be carried out in two steps, especially when the liquor contains an oxidant. Thus, the pulp may be brought into suspension in the liquor at room temperature (20° C.) or higher to promote the reaction of the oxidant on the pulp and thus to facilitate the procurement of a final product of low solution viscosity, whereupon the suspension may be cooled to room temperature (20° C.) or to below room temperature to enhance its solubilizing effect on the pentosans and thus to make possible the production of a final product of maximum alpha cellulose content. The cooling of the pulp suspension is preferably effected after the oxidant has been substantially consumed. To instance this sort of procedure, I may cite the admixture of a pulp with a heated 15% caustic soda solution containing about 8% hypochlorite bleach, based on the weight of pulp, to produce a pulp suspension at, say, 40° C., whereafter, with the bleach practically consumed by reaction on the pulp, the suspension may be cooled to 20° C. or lower and kept thereat for the desired period of time.

What I claim is:

1. A process which comprises suspending pre-liberated hardwood pulp in a mercerizing liquor containing an oxidant for about two to eight hours or more, washing the mercerized pulp free from mercerizing liquor, treating the washed pulp with caustic soda to form soda cellulose, and treating the soda cellulose without ageing with carbon bisulphide to form viscose.
2. A washed, mercerized hardwood pulp having an alpha cellulose content of at least about 94%, a pentosan content not exceeding about 1.5%, and a solution viscosity sufficiently low to

5 permit such pulp to be converted directly into cellulose xanthate and without intermediate aging of the soda cellulose prepared therefrom, said pulp being further characterized by an average fiber length much shorter than that of spruce sulphite pulp and the quicker convertibility of its shorter fiber units into cellulose xan-

thatate and said pulp being prepared according to a process which comprises suspending preliberated hardwood pulp in a mercerizing liquor containing an oxidant for about two to eight hours or more and washing the mercerized pulp free from mercerizing liquor.

GEORGE A. RICHTER.